

## UNITED STATES PATENT OFFICE

CAMILLE DREYFUS, OF NEW YORK, N. Y.

YARN, FABRIC, PLASTIC, ETC.

No Drawing.

Application filed March 30, 1926. Serial No. 98,815.

Heretofore it has been impractical to use artificial yarns, fabrics, films, etc., made of nitrocellulose because of the high inflammability and explosibility of the nitrocellulose. 5 Altho it is true that yarns, fabrics, etc., are made from nitrocellulose, they are not utilized in that form. They are subsequently denitrated and re-converted to cellulose. Because of these undesirable properties of nitrocellulose it has been impossible to use nitrocellulose silk, etc., and the use of celluloid and plastic compositions and films containing nitrocellulose compounds has been restricted in a great degree. Thus they cannot 10 be used where relatively high temperatures are met with or where they would be subjected to electrical discharges, to friction, etc.

The applicant has now discovered that the various nitrocellulose compounds can be 20 treated to materially lessen their inflammability without affecting appreciably their desirable properties. He has discovered that if a yarn, textile, film, fabric or plastic mass, containing or consisting of nitrocellulose, is 25 weighted the inflammability of the same is greatly reduced. In the case of yarns, films, fabrics and the like, this weighting of the nitrocellulose, with the consequent reduction in inflammability, does away with the necessity of denitrating. In the case of celluloid and other plastics containing or consisting of 30 nitrocellulose their field of usefulness is greatly increased.

As examples of the process which may be 35 employed to weight nitrocellulose the following may be given:

The weighting may be accomplished by treating the nitrocellulose material with a solution of a salt or salts of tin, zinc, tungsten or aluminum, for instance, stannic chloride or any other suitable salt for weighting, fixing the tin or other metal therein by a subsequent treatment with a solution of sodium phosphate or sodium silicate or both or 45 any other salt or salts suitable for fixing the metal salt or salts used in the first treatment. Or the nitrocellulose material may first be gelled by treatment with a dilute solution of formic or acetic acids or any other suitable 50 gelling, softening or swelling agent in suit-

able dilution or emulsion and then treated with a solution of stannic chloride, washed and the tin fixed therein by treating with a sodium phosphate or sodium silicate solution or both or any other salt or salts suitable for 55 fixing the metal salt or salts used in the first treatment. The swelling, gelling or softening agent in suitable dilution or emulsion may also be incorporated during the treatment with the tin chloride, or the tin salt 60 itself may be used in such a concentration and at such a temperature that it itself acts as a swelling agent.

The film, yarn, fabric or other article containing nitrocellulose can also be weighted 65 by treatment with tannic acid alone or by a treatment with tannic acid followed by a treatment with tartar emetic or by a tannic acid treatment followed by a treatment with a solution of stannic chloride. Any of the 70 usual methods used for weighting silk or artificial silk, which are suitable, also may be employed to weight the nitrocellulose.

The weighting of nitrocellulose fibres or fabrics removes not only the necessity of 75 denitrating the same in order to make them usable but it also improves the properties of such fabrics or articles in many other respects. Thus a circular knit fabric of nitrocellulose which fabric has been weighted will 80 have its tendency to "ladder" very greatly diminished—the greater the percentage of weighting the less the tendency to ladder. In a similar manner a weighted fabric entirely of nitrocellulose or a weighted mixed 85 fabric containing nitrocellulose fibres will lose the tendency to slip or shift due to the fact that the weighted fibres are enlarged and form a firmer contact with the adjacent fibres. The melting or rather the decomposition 90 point of fabrics containing weighted nitrocellulose is raised as a result of the weighting and the inflammability of the nitrocellulose is lowered making it even possible for the fabric to be ironed. It has also been 95 discovered that the tendency of nitrocellulose fabrics and yarns to become delustered when dyed at elevated temperatures is appreciably lessened when such a fabric or yarn has been 100 previously weighted. Nitrocellulose articles

which have been weighted show another marked improvement over the unweighted nitrocellulose articles. The latter are very difficultly dyed whereas the former are very easily dyed when subjected to a dyeing operation with various dyestuffs.

The improved properties of the nitrocellulose products as above referred to are independent of any particular weighting agent or agents and of the process employed in the application of the weighting agent to the nitrocellulose material.

The above examples are merely illustrative and should not be construed as limitative. The invention should be considered as limited only by the scope of the appended claims. The term "fabric" where used in the claims is to be construed as including textile or other finished articles such as garments, stockings, etc., and fabrics made from weighted nitrocellulose yarns.

What I claim and desire to secure by Letters Patent is:

1. An improved product comprising a nitrocellulose compound which is weighted with an insoluble metallic salt.
2. An improved product comprising a nitrocellulose compound which is weighted with an insoluble tin salt.
3. An improved product comprising a nitrocellulose compound weighted with a tin salt, fixed therein as tin phosphate.
4. A new and improved fabric containing nitrocellulose weighted with an insoluble metallic salt.
5. A new and improved fabric containing nitrocellulose fibres weighted with an insoluble tin salt.
6. A new and improved fabric containing nitrocellulose fibres weighted with a tin salt, which is present therein as tin phosphate.
7. A non-laddering or difficultly laddering circular knit fabric which contains nitrocellulose fibres weighted with an insoluble metallic salt.
8. A non-laddering or difficultly laddering circular knit fabric containing nitrocellulose fibres weighted with tin phosphate.
9. A non-slipping or difficultly slipping mixed fabric containing nitrocellulose fibres with an insoluble metallic salt thereon.
10. A non-slipping or difficultly slipping mixed fabric containing nitrocellulose fibres having tin phosphate thereon.
11. A plastic composition containing nitrocellulose weighted with an insoluble metallic salt.

In testimony whereof, I have hereunto subscribed my name.

CAMILLE DREYFUS.